

## UNITED STATES PATENT OFFICE.

LYALL ZICKRICK, OF CHICAGO, ILLINOIS, ASSIGNOR TO WESTERN ELECTRIC COMPANY, INCORPORATED, OF NEW YORK, N. Y., A CORPORATION OF NEW YORK.

## MAGNETIC MATERIAL AND METHOD OF PRODUCING IT.

No Drawing.

Application filed March 25, 1925. Serial No. 18,324.

This invention relates to magnetic materials and methods of producing them, and has for its object the production by a simplified and inexpensive method of a relatively cheap, brittle magnetic material having improved desirable magnetic characteristics and which may be readily reduced to a finely divided form.

The invention is of particular advantage in the production of magnet cores, particularly loading coil cores of the so-called "dust" type, such as are described in Patent No. 1,297,126, issued to Gustaf W. Elmen on March 11, 1919, and other patents therein referred to; but it will be apparent from the following description that the material may be put to other uses as will be indicated hereinafter.

The present invention is broadly characterized by the incorporation with a magnetic material of a small percentage of an embrittling agent, such as antimony, for the purpose of hardening and embrittling the magnetic material without impairing the desirable magnetic characteristics of the material. Hardened magnetic material so obtained may be easily pulverized in a suitable mill after which it may be used in the manufacture of cores for loading coils and other apparatus. The invention can be applied to any of the magnetic materials, but is of particular use with iron and nickel-iron.

The preferred method of producing the finely divided magnetic material in accordance with the invention is to preliminarily melt it and then incorporate a small amount of antimony with the melted material. The resulting alloy is then poured, preferably in a shallow mold, and allowed to solidify. It is then found to be in a porous, brittle condition after which it may be preliminarily broken up in a hammer mill and then reduced to finely divided form, preferably in the type of machine known as a "ball mill."

Where a good grade of commercial iron is employed, good results are obtained by employing from about 1.75% to about 15% of antimony. There may be other amounts of antimony which will give good results, but in the experiments on which the present invention is based, the best results seem to be within the range given. An iron-antimony alloy containing 1.75% antimony is

somewhat difficult to grind, but alloys containing as much as 4% of antimony can be reduced to finely divided form in the manner described in the preceding paragraph with very little difficulty. In regard to the magnetic properties of the alloy, the magnetic permeability seems to be somewhat greater and hysteresis losses somewhat less with smaller percentages of antimony. The magnetic characteristics of the material, however, will be more fully referred to in a following paragraph.

Where magnetic alloys composed of iron and other materials are employed the best results will be obtained by employing a different percentage of antimony than when iron alone is used. As an example, where antimony is to be added to a nickel-iron alloy for the purpose of embrittling it, a satisfactory embrittling effect is not obtained with a percentage of antimony substantially less than 5%. At the same time it is found that substantially more than 8% of antimony is apt to cause a considerable decrease in the high magnetic permeability of the nickel-iron and for this reason where the high magnetic permeability of nickel-iron at low magnetizing forces is sought to be retained, it is not desirable to employ more than 8% of the embrittling agent. For mechanical purposes the best amount of antimony seems to be about 6½%, but where the electrical or magnetic characteristics of the material are sought to be varied, a somewhat different percentage may be used and a satisfactory embrittling effect obtained.

When the finely divided magnetic material has been obtained it may be employed in various manners where its magnetic properties can be utilized. This use may entail the insulating of the particles from each other which may be accomplished by incorporating the particles with some insulating material of either the organic or inorganic type which material may be either plastic or non-plastic, depending upon the manner in which the resulting mixture is to be employed. Where the dust is compounded with a plastic insulator it may be treated in the manner described in the application of William Fondiller, Serial No. 741,041, filed October 1, 1924. The use therein described is generally termed continuous loading and as described in such application it may be

accomplished by compounding the magnetic particles with a plastic material and extruding the resulting mixture onto a conductor or by incorporating the particles with an insulating enamel before the application thereof to the conductor, and then baking the enamel to cause the mixture to adhere to the conductor.

The iron-antimony particles are of particular advantage in the production of magnet cores, particularly those for use in loading coils. These cores may be made in the manner described in the patent to Elmen mentioned above and the other patents there-  
15 in referred to, the method being briefly to coat the particles with insulating material, preferably shellac, and then by great pressure to force the particles into the form of a core or into a plurality of solid portions  
20 which may be assembled to form a core.

The magnetic properties of the material embodying the features of the present invention may be apparent from a consideration of the characteristics of a specific loading coil core formed thereof during the experimental work in connection with this invention. In this particular instance a good grade of commercial iron was melted in an induction furnace and then 6% of  
25 antimony was added thereto. The resulting alloy was poured into a flat mold and allowed to solidify after which it was broken up and reduced to finely divided form in the manner described hereinbefore. When the  
30 particles were sufficiently fine to pass through an 80-mesh screen they were tumbled with a quantity of feathered zinc in order to form a zinc coating thereon, the details of this step of the process being car-  
35 ried on in the manner described in Patent No. 1,292,206, issued January 21, 1919, to J. C. Woodruff. The zinc coated particles were then insulated with shellac and pressed into the form of a homogeneous solid with a  
40 pressure of 200,000 pounds per square inch, the details of these steps being substantially as described in Patent No. 1,274,952, issued August 6, 1918 to J. B. Speed. The core produced in this manner was then tested  
45 and found to have a permeability of 44 at a flux density of 17 lines and a frequency of 900 cycles. Under the same conditions the hysteresis loss was 7.3 ohms per henri, while the power loss due to eddy currents was as

low as 1.5 ohms per henri of inductance. It is understood, however, that this example is simply illustrative of one particular embodiment of the invention and that other materials, such as aluminum, silicon and tin, may be employed in other articles and may be produced by other processes and therefore the invention is to be limited only by the scope of the appended claims.

What is claimed is:

1. A method of producing magnetic material, which consists in alloying antimony with a magnetic material, and reducing the resulting product to finely divided form. 65
2. As a new article of manufacture, an alloy of magnetic material and antimony reduced to finely divided form. 70
3. A magnetic material comprising an alloy of iron and antimony reduced to finely divided form. 75
4. A method of producing magnetic material, which consists in alloying antimony with an iron-nickel alloy, and reducing the resulting product to a finely divided form.
5. A method of embrittling magnetic materials, which consists in alloying antimony therewith. 80
6. A method of embrittling ferrous magnetic alloys, which consists in alloying antimony therewith. 85
7. A method of embrittling iron-nickel alloys, which consists in alloying antimony therewith. 90
8. A magnetic material comprising from 1.75 to 15% antimony and the remainder principally iron. 95
9. A magnetic alloy comprising from 5 to 8% antimony alloyed with a magnetic material. 100
10. A method of producing magnetic material, which consists in alloying an embrittling agent with a magnetic substance.
11. A method of producing magnetic material, which consists in alloying a metallic embrittling agent with magnetic alloys of nickel and iron.
12. A method of producing magnetic material, which consists in alloying a metallic embrittling agent with magnetic alloys of nickel and iron.

In witness whereof, I hereunto subscribe my name this eleventh day of March A. D., 1925.

LYALL ZICKRICK.